

## UNITED STATES PATENT OFFICE

2,391,468

## METHOD OF MAKING MANIFOLDS

Robert Long, Muskegon, Mich., assignor to American Porcelain Enamel Company, Muskegon, Mich., a corporation of Michigan

No Drawing. Application February 10, 1942,  
Serial No. 430,239

2 Claims. (Cl. 117—129)

The present invention relates to a manifold capable of withstanding oxidation at the temperatures to which it is subjected in the operation of internal combustion engines, and has to do with the method of making such a manifold.

Prior manifolds such as are in use with airplane engines are unsatisfactory in that these manifolds must be frequently replaced because of oxidation thereof due to the hot gases passing through them. The exhaust manifolds of air cooled airplane engines operate at temperatures of the order of 1250° F. to 1500° F. which is sufficient to cause oxidation of present known manifolds. Stainless steel is the most common material in use today for the purpose, but this material is expensive and is not capable of completely withstanding oxidation at the temperatures to which the manifold is subjected by the products of combustion of an internal combustion engine.

It is an object of my invention to provide a manifold made of metal, preferably of ordinary wrought steel, having a non-metallic or vitreous coating which will not be destroyed by the hot gases encountered in the operation of internal combustion engines.

A further object is to provide an impervious vitreous coating on a manifold which prevents the oxidizing components of gases from attacking and oxidizing the metal of which the manifold is made.

A further object is the provision of a method of coating a manifold to prevent oxidization thereof.

The coating of my invention is impervious to gases and is resistant to high temperatures so that it is not essential that metal of which the manifold is made be of good grade or expensive character. Entirely satisfactory results may be attained by the use of wrought steel. Further, the coating is economical to manufacture and may be applied to a wrought metal tube or the like with a minimum of effort and expense.

It will be understood that the coating may be employed in many other instances in which it is desired to protect a surface against the deteriorating effects of high temperatures and oxidizing components of gases and the like.

Now in order to acquaint those skilled in the art with the manner of utilizing my invention I shall describe a specific embodiment of my invention as it relates to the manufacture of a manifold.

An ordinary wrought steel or other metal tubing or the like suitable for use as a manifold is first pickled to remove all grease, oil, and rust and the like. In order to remove the grease

and oil the steel tube may be placed in a solution of any known commercial cleaner. I prefer to use a solution comprising 3.0-3.3% sodium oxide and placing the tube therein for about 5 to 25 minutes, the solution being maintained at boiling temperature. Thereafter the rust and scale may be removed by depositing the steel tube in a solution of sulphuric acid of a strength of 6 to 7% and at a temperature of 150° F. for about 15 minutes. The acid is then rinsed off and the steel tube next neutralized to remove all traces of acid. This may be accomplished by placing the steel tube in a neutralizer solution of borax and soda ash for about 5 minutes. The strength of this solution preferably is 0.25% sodium oxide and should be at a temperature of about 170-180 degrees F. Other cleaning methods or ingredients may be employed if desired.

A coating for the steel tube is made up as follows:

A first frit is made in accordance with the following formula and in about the amounts of the identified components or ingredients as follows:

|    |                   |         |              |
|----|-------------------|---------|--------------|
| 25 | Feldspar          | 185     | lbs.         |
|    | Quartz            | 209 1/4 | lbs.         |
|    | Razorite          | 209     | lbs.         |
|    | Soda ash          | 43 1/2  | lbs.         |
|    | Sodium nitrite    | 34 1/4  | lbs.         |
| 30 | Fluorspar         | 44 3/4  | lbs.         |
|    | Manganese dioxide | 14 1/2  | lbs.         |
|    | Cobalt oxide      | 4       | lbs. 13 ozs. |
|    | Nickel oxide      | 3       | lbs. 12 ozs. |

The above amounts of these several ingredients are calcined or roasted together to render the frit insoluble in water. Calcining is well known in the art and is also frequently referred to as fritting. Preferably the frit is ground or broken up after calcining so that it may be readily handled and weighed.

A second frit is made in accordance with the following formula and in about the amounts of the identified components or ingredients as follows:

|    |                   |               |      |
|----|-------------------|---------------|------|
| 50 | Razorite          | 195 1/4       | lbs. |
|    | Feldspar          | 217 1/2       | lbs. |
|    | Quartz            | 140 1/2       | lbs. |
|    | Soda ash          | 52            | lbs. |
|    | Sodium nitrite    | 25            | lbs. |
|    | Fluorspar         | 43 1/2        | lbs. |
|    | Zircon            | 33 3/4        | lbs. |
|    | Calcium carbonate | 24 1/4        | lbs. |
| 55 | Manganese dioxide | 11            | lbs. |
|    | Nickel oxide      | 4 lbs. 10 oz. |      |
|    | Cobalt oxide      | 3             | lbs. |

This frit is made up in the same manner as the first referred to frit, i. e., the given amounts of the several ingredients are calcined to render the frit insoluble in water.

After the above two frits have been prepared, I take nine parts of the first frit by weight to one part of the second frit by weight and mill them together with a mill addition comprising the following components or ingredients which are added to the nine parts of the first frit and the one part of the second frit in the following percentages of the sum of the parts of frits 1 and 2.

|                       | Per cent |
|-----------------------|----------|
| Clay (enameling clay) | 7.0      |
| Feldspar              | 10.5     |
| Borax                 | .75      |
| Sodium nitrite        | .125     |
| Magnesium carbonate   | .125     |
| Water                 | 50.0     |

The mixture is then ground in the milling apparatus until an enamel is formed of which about 6 or 7% will remain on a 200 mesh screen.

After the frits 1 and 2 and the mill addition have been ground to a fineness of the character above noted, water is added to the enamel until the amount deposited upon a test sheet is one ounce per square foot, dry. This refers to the actual weight of enamel per square foot on the tube after all the water has been deleted. After the enamel has been brought to this consistency, the steel tubes are coated preferably by dipping them in the enamel. The tubes are then preferably positioned in a suitable dryer to remove all water from the coating. Thereafter, the steel tubes are placed in a suitable furnace and burned at a temperature of the order of 1620 degrees F. for about 8 or 9 minutes. The tubing is then ready for use as a manifold. If desired the coating may be applied by other than dipping. Preferably both the inner and outer surfaces are coated but in certain instances it may be desired or only essential to coat a single surface. This may be accomplished in any suitable manner.

A chemical analysis of the coating after the burning step above referred to is as follows:

|                   | Per cent |
|-------------------|----------|
| Silica            | About    |
| Alumina           | 50.2     |
| Boric oxide       | 6.7      |
| Sodium oxide      | 13.3     |
| Potassium oxide   | 17.0     |
| Calcium oxide     | 3.6      |
| Manganese dioxide | 6.7      |
| Nickel oxide      | 1.6      |
| Cobalt oxide      | 0.4      |
| Zirconium dioxide | 0.6      |
|                   | 0.1      |

It is calculated that there is about a 0.3% ignition loss as a result of the burning step.

The coating thus provided is impervious to oxidizing components of gases and the like at temperatures of the order of 1250° F. to 1500° which is the range of temperatures to which air cooled exhaust manifolds of internal combustion engines are heated. This temperature range of air cooled exhaust manifolds of airplane engines represents the maximum temperature range to which manifolds of internal combustion engines are heated and it will be observed therefore that my invention is suitable for other types and characters of manifolds. The finished coating is of a vitreous character and of dark blue color. The coating is hard and brilliant. I have found that

the finished coating will satisfactorily withstand a temperature of the order of 1500° F. and further is not readily damaged by temperatures of the order employed in the burning step of my method.

It will appear that I have provided a manifold which is capable of withstanding the temperatures to which it is heated by the hot gases of an internal combustion engine. Also the coating prevents oxidation of the manifold by the surrounding air at the temperature to which it is heated by the hot gases or products of combustion of an internal combustion engine. It will be understood that the composition of the coating of my invention is not limited to use with a manifold, but may be readily applied to any surface which it is desired to protect from the oxidizing effects of gases and from deteriorating effect of high temperatures.

20 I claim:

1. The method of treating a metal manifold which comprises, forming a first frit of the following ingredients:

|    |                   |                     |
|----|-------------------|---------------------|
| 25 | Feldspar          | About 185 lbs.      |
|    | Quartz            | About 209 1/4 lbs.  |
|    | Rasorite          | About 209 lbs.      |
|    | Soda ash          | About 43 1/2 lbs.   |
|    | Sodium nitrite    | About 34 1/4 lbs.   |
| 30 | Fluorspar         | About 44 3/4 lbs.   |
|    | Manganese dioxide | About 14 1/2 lbs.   |
|    | Cobalt oxide      | About 4 lbs. 13 oz. |
|    | Nickel oxide      | About 3 lbs. 12 oz. |

35 forming a second frit of the following ingredients:

|    |                   |                     |
|----|-------------------|---------------------|
| 35 | Rasorite          | About 195 1/4 lbs.  |
|    | Feldspar          | About 217 1/2 lbs.  |
|    | Quartz            | About 140 1/2 lbs.  |
| 40 | Soda ash          | About 52 lbs.       |
|    | Soda nitrate      | About 25 lbs.       |
|    | Fluorspar         | About 43 1/2 lbs.   |
|    | Zircon            | About 33 3/4 lbs.   |
|    | Calcium carbonate | About 24 1/4 lbs.   |
| 45 | Manganese dioxide | About 11 lbs.       |
|    | Nickel oxide      | About 4 lbs. 10 oz. |
|    | Cobalt oxide      | About 3 lbs.        |

50 taking nine parts by weight of the first frit with one part by weight of the second frit and milling said parts with a mill addition comprising the following components in the following percentages of the sum of said parts:

|                     | Per cent   |
|---------------------|------------|
| Clay                | About 7    |
| Feldspar            | About 10.5 |
| Borax               | About .75  |
| Sodium nitrite      | About .125 |
| Magnesium carbonate | About .125 |
| Water               | About 50   |

55 to form an enamel, coating at least one surface of said manifold with said enamel, drying said coating, and burning said coating.

2. The method of treating a wrought steel manifold which comprises, forming a first frit of the following ingredients:

|    |                   |                     |
|----|-------------------|---------------------|
| 55 | Feldspar          | About 185 lbs.      |
|    | Quartz            | About 209 1/4 lbs.  |
|    | Rasorite          | About 209 lbs.      |
|    | Soda ash          | About 43 1/2 lbs.   |
|    | Sodium nitrite    | About 34 1/4 lbs.   |
|    | Fluorspar         | About 44 3/4 lbs.   |
|    | Manganese dioxide | About 14 1/2 lbs.   |
|    | Cobalt oxide      | About 4 lbs. 13 oz. |
|    | Nickel oxide      | About 3 lbs. 12 oz. |

forming a second frit of the following ingredients:

|                   |                              |
|-------------------|------------------------------|
| Razorite          | About 195 $\frac{1}{4}$ lbs. |
| Feldspar          | About 217 $\frac{1}{2}$ lbs. |
| Quartz            | About 140 $\frac{1}{2}$ lbs. |
| Soda ash          | About 52 lbs.                |
| Sodium nitrite    | About 25 lbs.                |
| Fluorspar         | About 43 $\frac{1}{2}$ lbs.  |
| Zircon            | About 33 $\frac{3}{4}$ lbs.  |
| Calcium carbonate | About 24 $\frac{1}{4}$ lbs.  |
| Manganese dioxide | About 11 lbs.                |
| Nickel oxide      | About 4 lbs 10 oz.           |
| Cobalt oxide      | About 3 lbs.                 |

taking nine parts by weight of the first frit with one part by weight of the second frit and milling said parts with a mill addition comprising the

following components in the following percentages of the sum of said parts:

|                     | Per cent   |
|---------------------|------------|
| Clay                | About 7    |
| Feldspar            | About 10.5 |
| Borax               | About .75  |
| Sodium nitrite      | About .125 |
| Magnesium carbonate | About .125 |
| Water               | About 50   |

10 to form an enamel of a fineness so that the major portion thereof is passable through a 200 mesh screen, adding water to said enamel until the amount deposited on a test sheet is one ounce per square foot, dry, depositing a coating of said enamel on at least one surface of said manifold, drying said coating and burning said coating at a temperature of about 1620° F. for about nine minutes.

ROBERT LONG.